

# UNITED STATES PATENT OFFICE.

ALMER McDUFFIE McAFFEE, OF NEW YORK, N. Y., ASSIGNOR TO GULF REFINING COMPANY, OF PITTSBURGH, PENNSYLVANIA, A CORPORATION OF TEXAS.

## PROCESS OF SATURATING OILS.

1,277,328.

Specification of Letters Patent. Patented Aug. 27, 1918.

No Drawing.

Application filed December 8, 1915. Serial No. 65,289.

To all whom it may concern:

Be it known that I, ALMER McDUFFIE McAFFEE, a citizen of the United States, residing at New York, in the county of New York and State of New York, have invented certain new and useful Improvements in Processes of Saturating Oils, of which the following is a specification:

This invention relates to processes of saturating oils; and it comprises a method of converting lower grade kerosene into higher grade kerosene wherein kerosene is warmed with aluminum chlorid at a relatively low temperature for a time, the temperature being below that at which aluminum chlorid will exercise any violent breaking down action upon the hydrocarbons of such oil but being sufficient to permit such aluminum chlorid to exert what may be termed a saturating and stabilizing action; a temperature which is in the neighborhood of 150° F. or between 150° F. and 212° F.; the warming with the aluminum chlorid being continued until a desired degree of saturation and internal change, with corresponding improvement, is accomplished; all as more fully hereinafter set forth and as claimed.

Petroleum oils and products are composed mainly or exclusively of various hydrocarbons of different boiling points. While these hydrocarbons, which are bodies consisting of hydrogen and carbon in chemical union, are very many in number and differ among themselves in chemical and physical properties, for the present purposes they may be divided into two well-known classes, the saturated hydrocarbons and the unsaturated hydrocarbons. The former are those which contain enough hydrogen to saturate all the chemical combining power of the carbon which they also contain, while the latter are those in which the carbon has some of its affinities unsaturated and is therefore in condition to enter into further union with oxygen and other bodies. The unsaturated hydrocarbons are presumed to owe their reactive nature to the presence of "double linkage" or "triple linkage" as the case may be; to the presence of pairs of adjacent carbon atoms united together by two or more bonds instead of union by a single bond only. The saturated hydrocarbons are relatively stable bodies; the unsaturated are relatively unstable. The odor of unsaturated hydrocarbons is also markedly more offensive than

that of the saturated hydrocarbons. Corresponding to this chemical difference between the two classes is a market difference in values. In all commercial petroleum products those which contain any substantial amount of unsaturated hydrocarbons are of lower grade than those which are free, or relatively free, of such unsaturated hydrocarbons. The unsaturated hydrocarbons occurring in kerosene are of course themselves oils of the general character of kerosene and, except as regards stability, they do not differ materially from the saturated hydrocarbons or oils which they accompany. They are hardly to be regarded as impurities; they are simply oils of less desirable character. If they be removed from the oily body, as is practicable by the use of sulfuric acid, etc., there is a resulting loss of oil.

Aluminum chlorid ( $AlCl_3$ , or  $Al_2Cl_6$ ) is a material capable of exercising sundry energetic reactions with the hydrocarbons which compose petroleum oil, and of modifying their character in many ways. On heating a high-boiling petroleum oil, such as lubricating oil, a gas oil or solar oil, kerosene, etc., with aluminum chlorid, the latter, under proper conditions, will convert the whole of such high boiling oil into lower boiling oils of the nature of gasolene, with perhaps 10 or 15 per cent. loss as gas and coke. All the distillation products of such an action will be found to be of saturated nature whatever was the nature, in this respect, of the original high boiling oil treated; by distilling a highly unsaturated gas oil, it may be converted practically wholly into gasolene and this gasolene will all be of saturated nature.

I have found that by operating at a sufficiently low temperature, instead of working at the boiling temperature just described, I can wholly obviate the stated converting action while still retaining the saturating action and that this may be utilized in bettering the quality of kerosene without the loss of oil incidental to other methods of purifying kerosene. In other words, I can take a kerosene oil containing unsaturated hydrocarbons and warm it (as distinguished from heating at any high temperature) with aluminum chlorid and produce a saturation of the unsaturated constituents without production of lower boiling oils. In this action the unsaturated oils are simply transformed

60

65

70

75

80

85

90

95

100

105

110

into saturated oils without material loss in volume or weight such as occurs in removing unsaturated compounds with sulfuric acid. The temperatures necessary for this action are around 150° F. Below that temperature the saturating action becomes slower, while at temperatures materially above, say 212° F., the action may go so far as to produce some lower boiling oil. With kerosene, any production of lower boiling oils is highly undesirable as unduly lowering the flash point.

In a practical embodiment of my process of treating kerosene or illuminating oil to improve its color and stability, as well as its burning qualities, I may take a low grade kerosene containing unsaturated hydrocarbons or oils and warm it to about 150° F. with a suitable amount of anhydrous aluminum chlorid, say 5 per cent. The oil must be dry, since any moisture deteriorates or destroys the activity of the aluminum chlorid. Freshly distilled illuminating oils are sufficiently dry. Older oils are best dried with a current of air. The aluminum chlorid does not dissolve to any great extent in the cold oil although its solubility increases on warming to the temperature stated; and in order to maintain efficient contact between the oil and aluminum chlorid, stirring or agitation is resorted to. Different oils require somewhat different temperatures and times of action; but as a rule around 150° F. for four to six hours will be found satisfactory. The time element depends largely upon the amount of improvement which may be desired (i. e., of transformation of unsaturated groups present) in the grade of oil. The progress of the action may be followed by removing portions of oil from time to time, cooling, filtering through paper and testing with iodin solution. Unsaturated hydrocarbons have the power of absorbing iodin and the progressive diminution in the amount of iodin absorbed indicates the progressive diminution in the proportion of unsaturated components present in the oil. The operation may be arrested when the iodin test shows a desired amount of improvement. With any given oil it is of course not necessary to test every batch treated. The best operating temperature for any given oil can be adjudged in much the same way. It is desirable to work at as high a temperature (for the sake of speed) as possible but without any material production of low boiling oils (that is, gasolete and the like) as indicated by observing the flash point.

As stated, in the case of illuminating oils,

lubricating oils and the like, it is highly undesirable to lower the flash point.

When the operation has been carried as far as may be desired, as for instance to the point where the iodin number ceases to diminish rapidly, warming and stirring may be interrupted and the mass allowed to cool. The aluminum chlorid then for the most part separates out as a heavy sludge. The sludge may be removed and used to treat successive new batches of oil. Its activity steadily diminishes with reuse and it is finally converted into a granular inactive coky mass. From this it may be recovered for reuse by appropriate methods.

The oil from which the chlorid sludge has separated still carries a little aluminum chlorid in suspension. From this it may be freed by agitating with a little sulfuric acid or by filtration through fullers' earth; or both. Or the oil may be subjected to a current of steam.

The oil treated as thus described differs from the original oil in being colorless or of a less color; and in being permanent on keeping. It does not tend to absorb oxygen from the air; and its burning qualities are improved.

In my application Serial No. 224038, filed March 22, 1918, filed as a continuation of application Serial No. 792615, filed September 30, 1913, I have described and claimed the process of treating and improving petroleum hydrocarbons generally and lubricating oils specifically, such process involving the use of aluminum chlorid. The present application is directed to a process of treating and improving kerosene.

What I claim is:

1. The process of decolorizing and improving kerosene, which comprises warming such kerosene with aluminum chlorid at a temperature around 150° F.

2. The process of stabilizing, decolorizing and deodorizing illuminating oils containing unsaturated oils, which comprises warming such an oil with anhydrous aluminum chlorid at a temperature sufficient to transform such unsaturated oils into saturated oils while insufficient to cause a substantial lowering of the original flash point of such illuminating oil.

3. The process of decolorizing and improving kerosene which comprises warming the same with aluminum chlorid at a temperature insufficient to produce any substantial lowering of the boiling point.

In testimony whereof, I affix my signature.

ALMER McDUFFIE McAFFEE.